# EUROPEAN PATENT SPECIFICATION

(11) **EP 0 588 429 B1**
(45) Date of publication and mention of the grant of the patent: **25.03.1998**
(21) Application number: 93202640.4
(22) Date of filing: 10.09.1993
(51) Int. Cl.: C10L 1/14, C10L 10/00

(54) **Gasoline composition**
Benzinzusammensetzung
Composition d'essence

(30) Priority: 14.09.1992 EP 92308319
(43) Date of publication of application: 23.03.1994
(73) Proprietor: SHELL INTERNATIONALE RESEARCH MAATSCHAPPIJ B.V., 2596 HR Den Haag (NL)
(72) Inventor: Graham, Joseph, Wirral, Merseyside, L63 0NE (GB); Van Es, Cornelis, Adisham, Kent CT3 3LG (GB)

(56) References cited:
- EP-A- 0 290 088
- EP-A- 0 384 605
- EP-A- 0 526 129
- WO-A-92/02601
- GB-A- 2 261 441
- US-A- 5 006 130

## Description

This invention relates to gasoline compositions comprising a major amount of a gasoline suitable for use in spark-ignition engines and a minor amount of at least one additive, and to additive concentrates suitable for addition to gasoline to prepare such gasoline compositions.

EP-A-290 088 discloses gasoline compositions comprising a major amount of a gasoline suitable for use in spark-ignition engines, and a minor amount of a polyalphaolefin having a viscosity at 100°C from 2 x 10⁻⁶ to 2 x 10⁻⁵ m²/s (2 to 20 centistokes), preferably a hydrogenated oligomer containing 18 to 80 carbon atoms derived from an alphaolefinic monomer containing from 8 to 12 carbon atoms, and optionally minor amounts of an oil-soluble aliphatic polyamine and/or an alkali metal or alkaline-earth metal salt of a succinic acid derivative having a polyolefin substituent on at least one of its carbon atoms and/or a polyolefin derived from a C₂ to C₆ monomer having a number average molecular weight (Mₙ) between 500 and 1500.

US Patent No. 3,901,665 discloses liquid hydrocarbon fuel compositions characterised by improved anti-icing and carburetor detergency comprising
A. a major amount of a liquid hydrocarbon fuel comprising hydrocarbons boiling in the gasoline range, and based on the weight of said fuel
B. about from 0.01 to about 0.06 percent by weight of a 3- or 4-carbon olefin, preferably polyisobutylene, having a molecular weight of from about 400 to about 1400, preferably about 400 to about 900, and
C. from about 0.008 to about 0.016 percent by weight of a polyoxyalkylene compound of the formula wherein R is alkyl of 1 to 20 carbon atoms, preferably 10 to 18 carbon atoms, and x has an average value of 4 to 20; and additive compositions consisting essentially of B and C.

US Patent No. 3,658,494 discloses fuel compositions comprising a major amount of at least one normally liquid fuel and a minor amount of an additive combination soluble in said fuel, the additive combination comprising (a) at least one oxy compound which is a monoether of a glycol or polyglycol and (b) at least one fuel-soluble dispersant selected from the class consisting of esters, amides, imides, amidines, and amine salts of at least one substantially saturated carboxylic acid characterised by the presence within the acyl radical thereof of at least 30 aliphatic carbon atoms, the weight ratio of oxy compound to dispersant being about 0.1:1 to about 1:0.1, but preferably 0.1:1 to about 2.5:1. In the examples the oxy compounds used are ethylene glycol mono-n-butyl ether, dipropylene glycol monomethyl ether, triethylene glycol monoethyl ether, and ethylene glycol monophenyl ether.

EP-A-384 605 discloses a motor fuel composition which comprises a mixture of hydrocarbons boiling in the gasoline boiling range and additionally (1) the reaction product of a defined hydrocarbyl-substituted dibasic acid and a defined polyoxyalkylene diamine, (ii) a polymeric component which is a polyolefin polymer, copolymer, or the corresponding aminated or hydrogenated polymer or copolymer, or mixtures thereof, of a C₂₋₁₀ hydrocarbon, said polyolefin polymer or copolymer having a molecular weight in the range of 500 to 10,000; (iii) a polyalkylene glycol having a molecular weight in the range of 500-2000; and (iv) a lubricating oil. In relation to (ii) it is stated (Page 9 lines 39, 40) in general the olefin monomers from which the polyolefin polymer component is prepared are preferably unsaturated C₂₋₆ hydrocarbons. The polyalkylene glycol (iii) is said (Page 10 lines 39, 40) preferably to be selected from the group consisting of polyethylene glycol, polypropylene glycol and polybutylene glycol.

EP-A-526129 (published on 3 February 1993) discloses a fuel additive concentrate for controlling octane requirement increase in internal combustion engines comprising the reaction product of (i) polyamine and (ii) at least one acyclic hydrocarbyl substituted succinic acylating agent, and an unhydrotreated poly-alpha-olefin. Whilt EP-A-526 129 further and more specifically provides a fuel composition comprising a major amount of hydrocarbons in the gasoline boiling range, or hydrocarbon/oxygenate mixtures, or oxygenates containing a minor, but effective amount, of (a) a fuel additive comprising the reaction product of (i) polyamine and (ii) at least one acyclic hydrocarbyl substituted succinic acylating agent; (b) an unhydrotreated poly-alpha-olefin having a volatility of about 50% or less as determined by a test method described therein; (c) and optionally (A) a mineral oil having a viscosity index of less than about 90 and a volatility of 50% or less as determined by a test method described therein; (B) an antioxidant, or (C) a demulsifier, or (D) an aromatic hydrocarbon solvent, or (E) a corrosion inhibitor, or any combination of any two, three, four, or all five of components (A), (B), (C), (D) and (E), it is clearly an essential feature that the poly-alpha-olefin present is an unhydrotreated poly-alpha-olefin. The demulsifier (c) includes polyoxyalkylene glycols and oxyalkylated phenolic resins, and in particular mixtures of these.

It has now surprisingly been found that gasolines incorporating combinations of particular polyalphaolefins and particular polyoxyalkylene glycol derivatives can give surprisingly enhanced engine performance in terms of an advantageous combination of minimised engine inlet system deposits and minimised valve sticking.

According to the present invention there is provided a gasoline composition comprising a major amount of a gasoline suitable for use in spark-ignition engines, an amount of a polyalphaolefin having a viscosity at 100°C in the range 2 x 10⁻⁶ to 2 x 10⁻⁵ m²/s (2 to 20 centistokes), being a hydrogenated oligomer containing 18 to 80 carbon atoms derived from at least one alphaolefinic monomer containing from 8 to 16 carbon atoms, and an amount of a polyoxyalkylene compound selected from glycols, mono- and diethers thereof, having number average molecular weight (Mₙ) in the range 400 to 3000, the weight ratio polyalphaolefin: polyoxyalkylene compound being in the range 1:10 to 10:1, and the amount of the polyalphaolefin and the polyoxyalkylene compound together being in the range 100 to 1500 ppmw based on total composition.

The polyalphaolefins used in the gasoline compositions of the invention are primarily trimers, tetramers and pentamers, and synthesis of such materials is outlined in Campen et al., "Growing use of synlubes", Hydrocarbon Processing February 1982, Pages 75 to 82. The polyalphaolefin is preferably derived from an alphaolefinic monomer containing from 8 to 12 carbon atoms. Polyalphaolefins derived from decene-1 have been found to be very effective. The polyalphaolefin preferably has viscosity at 100°C in the range 6 x 10⁻⁶ to 1 x 10⁻⁵ m²/s (6 to 10 centistokes). Polyalphaolefin having a viscosity at 100°C of 8 x 10⁻⁶ m²/s (8 centistokes) has been found to be very effective.

The polyoxyalkylene compound may be represented by the formula wherein R¹ and R² independently represent hydrogen atoms or hydrocarbyl, preferably, C₁₋₄₀ hydrocarbyl, e.g. alkyl, cycloalkyl, phenyl or alkyl phenyl groups, each R independently represents an alkylene, preferably a C₂₋₈ alkylene, group, and n is such that Mₙ of the polyoxyalkylene compound is in the range 400 to 3000, preferably 700 to 2000, more preferably 1000 to 1500.

Preferably R¹ represents a C₈₋₂₀ alkyl group and R² represents a hydrogen atom. R¹ preferably represents a C₁₀₋₁₈ alkyl group, more preferably a C₁₂₋₁₅ alkyl group. R¹ may conveniently be a mixture of C₁₂₋₁₅ alkyl groups.

In formula I the groups R are preferably 1,2-alkylene groups.

Preferably each group R independently represents a C₂₋₄ alkylene group, e.g. an ethylene or 1,2-propylene group. Very effective results have been obtained using polyalkylene compounds wherein each group R represents a 1,2-propylene group.

The polyalphaolefin and the polyoxyalkylene compound together may advantageously be present in the gasoline composition in an amount in the range 100 to 1200 ppmw, preferably 100 to 600 ppmw, more preferably 150 to 500 ppmw, based on total composition.

The weight ratio polyalphaolefin:polyoxyalkylene compound in the gasoline composition is preferably in the range 1:8 to 8:1, more preferably 1:5 to 5:1. Weight ratios in the range 1:4 to 4:1 have been found to be very effective.

The gasoline compositions of the present invention desirably also contain a minor amount of at least one hydrocarbon-soluble ashless dispersant. The compounds useful as ashless dispersants generally are characterised by a "polar" group attached to a relatively high molecular weight hydrocarbon chain. The "polar" group generally contains one or more of the elements nitrogen, oxygen and phosphorus. The solubilising chains are generally higher in molecular weight than those employed with the metallic types, but in some instances they may be quite similar.

In general, any of the ashless dispersants which are known in the art for use in lubricants and fuels can be utilised in the gasoline compositions of the present invention.

In one embodiment of the present invention, the dispersant is selected from the group consisting of
(i) at least one hydrocarbyl-substituted amine wherein the hydrocarbyl substituent is substantially aliphatic and contains at least 8 carbon atoms;
(ii) at least one acylated, nitrogen-containing compound having a hydrocarbon-based substituent of at least 10 aliphatic carbon atoms made by reacting a carboxylic acid acylating agent with at least one amino compound containing at least one

   -NH-

   group, said acylating agent being linked to said amino compound through an imido, amido, amidine, or acyloxy ammonium linkage;
(iii) at least one nitrogen-containing condensate of a phenol, aldehyde and amino compound having at least one

   -NH-

   group;
(iv) at least one ester of a substituted carboxylic acid;
(v) at least one polymeric dispersant;
(vi) at least one hydrocarbon-substituted phenolic dispersant; and
(vii) at least one fuel soluble alkoxylated derivative of an alcohol, phenol or amine.

The hydrocarbyl-substituted amines used in the gasoline compositions of this invention are well known to those skilled in the art and they are described in a number of patents. Among these are U.S. Patents Nos. 3,275,554, 3,438,757, 3,454,555, 3,565,804, 3,755,433 and 3,822,209. These patents disclose suitable hydrocarbyl-substituted amines for use in the present invention including their method of preparation.

A typical hydrocarbyl-substituted amine has the general formula:

[AXN]ₓ[-N([-UN-]ₐ[-UQ]_{b})]_{y}R³ _{c}H_{1+2y+ay-c} (II)

wherein A is hydrogen, a hydrocarbyl group of from 1 to 10 carbon atoms, or hydroxyhydrocarbyl group of from 1 to 10 carbon atoms; X is hydrogen, a hydrocarbyl group of from 1 to 10 carbon atoms, or hydroxyhydrocarbyl group of from 1 to 10 carbon atoms, and may be taken together with A and N to form a ring of from 5 to 6 annular members and up to 12 carbon atoms; U is an alkylene group of from 2 to 10 carbon atoms, any necessary hydrocarbons to accommodate the trivalent nitrogens are implied herein, R³ is an aliphatic hydrocarbon of from 30 to 400 carbon atoms; Q is a piperazine structure; a is an integer of from 0 to 10; b is an integer of from 0 to 1; a+2b is an integer of from 1 to 10; c is an integer of from 1 to 5 and is an average in the range of 1 to 4, and equal to or less than the number of nitrogen atoms in the molecule; x is an integer of from 0 to 1; y is an integer of from 0 to 1; and x+y is equal to 1.

In interpreting this formula, it is to be understood that the R³ and H atoms are attached to the unsatisfied nitrogen valences within the brackets of the formula. Thus, for example, the formula includes sub-generic formulae wherein the R³ is attached to terminal nitrogens and isomeric subgeneric formulae wherein it is attached to non-terminal nitrogen atoms. Nitrogen atoms not attached to an R³ may bear a hydrogen or an AXN substituent.

The hydrocarbyl-substituted amines useful in this invention and embraced by formula II above include monoamines such as poly(propylene)amine, N,N-dimethyl-n-poly(ethylene/propylene)amine (50:50 mole ratio of monomers), poly(isobutene)amine, N,N-di(hydroxyethyl)-N-poly(isobutene)amine, poly(isobutene/1butene/2-butene)amine (50:25:25 mole ratio of monomers), N-(2-hydroxyethyl)-N-poly(isobutene)amine, N-(2-hydroxypropyl)-N-poly(isobutene)amine, N-poly(1-butene)-aniline, and N-poly(isobutene)-morpholine; and polyamines such as N-poly(isobutene) ethylene diamine, N-poly(propylene) trimethylene diamine, N-poly(1-butene) diethylene triamine, N',N'-poly(isobutene) tetraethylene pentamine, N,N-dimethyl-N'-poly(propylene), and 1,3-propylene diamine.

The hydrocarbyl-subsituted amines useful in the gasoline compositions of the invention also include certain N-amino-hydrocarbyl morpholines of the general formula:

R³N(A)UM (III)

wherein R³ is an aliphatic hydrocarbon group of from 30 to 400 carbons, A is hydrogen, a hydrocarbyl group of from 1 to 10 carbon atoms or hydroxyhydrocarbyl group of from 1 to 10 carbon atoms, U is an alkylene group of from 2 to 10 carbon atoms, and M is a morpholine structure. These hydrocarbyl-substituted aminohydrocarbyl morpholines as well as the polyamines described by formula II are among the typical hydrocarbyl-substituted amines used in preparing compositions of this invention.

A number of acylated, nitrogen-containing compounds having a hydrocarbon-based substituent of at least 10 aliphatic carbon atoms and made by reacting a carboxylic acid acylating agent with an amino compound are known to those skilled in the art. The acylating agent is linked to the amino compound through an imido, amido, amidine or acyloxy ammonium linkage. The hydrocarbon-based substituent of at least 10 aliphatic carbon atoms may be in either the carboxylic acid acylating agent derived portion of the molecule or in the amino compound derived portion of the molecule. Preferably, however, it is in the acylating agent portion. The acylating agent can vary from formic acid and it acylating derivatives to acylating agents having high molecular weight aliphatic substituents of up to 5,000, 10,000 or 20,000 carbon atoms. The amino compounds can vary from ammonia itself to amines having aliphatic substituents of up to 30 carbon atoms.

A typical class of acylated, nitrogen-containing compounds useful in the compositions of this invention are those made by reacting an acylating agent having an aliphatic substituent of at least 10 carbon atoms and a nitrogen compound characterised by the presence of at least one -NH- group. Typically, the acylating agent will be a mono- or polycarboxylic acid (or reactive equivalent thereof) such as a substituted succinic or propionic acid and the amino compound will be a polyamine or mixture of polyamines, most typically, a mixture of ethylene polyamines. The amine may also be a hydroxyalkyl-substituted polyamine. The aliphatic substituent in such acylating agents preferably averages at least 30 or 50 and up to 400 carbon atoms.

Illustrative hydrocarbon-based substituent groups containing at least ten aliphatic carbon atoms are n-decyl, n-dodecyl, tetrapropenyl, n-octadecyl, oleyl, chlorooctadecyl and triicontanyl. Generally, the hydrocarbon-based substituents are made from homo- or interpolymers (e.g., copolymers, terpolymers) of mono- and diolefins having 2 to 10 carbon atoms, such as ethylene, propylene, butene-1, isobutene, butadiene, isoprene, 1-hexene and, 1-octene. Typically, these olefins are 1-monoolefins. The substituent can also be derived from the halogenated (e.g., chlorinated or brominated) analogues of such homo- or interpolymers. The substituent can, however, be made from other sources, such as monomeric high molecular weight alkenes (e.g., 1-tetracontene) and chlorinated analogues and hydrochlorinated analogues thereof, aliphatic petroleum fractions, particularly paraffin waxes and cracked and chlorinated analogues and hydrochlorinated analogues thereof, white oils, synthetic alkenes such as those produced by the Ziegler-Natta process (e.g., poly(ethylene) greases) and other sources known to those skilled in the art. Any unsaturation in the substituent may be reduced or eliminated by hydrogenation according to procedures known in the art.

As used in this specification, the term "hydrocarbon-based" denotes a group having a carbon atom directly attached to the remainder of the molecule and having a predominantly hydrocarbon character within the context of this invention. Therefore, hydrocarbon-based groups can contain up to one non-hydrocarbon group for every ten carbon atoms provided this non-hydrocarbon group does not significantly alter the predominantly hydrocarbon character of the group. Those skilled in the art will be aware of such groups, which include, for example, hydroxyl, halo (especially chloro and fluoro), alkoxyl, alkyl mercapto and alkyl sulphoxy groups. Usually, however, the hydrocarbon-based substituents are purely hydrocarbyl and contain no such non-hydrocarbyl groups.

The hydrocarbon-based substituents are substantially saturated, that is, they contain no more than one carbon-to-carbon unsaturated bond for every ten carbon-to-carbon single bonds present. Usually, they contain no more than one carbon-to-carbon non-aromatic unsaturated bond for every 50 carbon-to-carbon bonds present.

The hydrocarbon-based substituents are also substantially aliphatic in nature, that is, they contain no more than one non-aliphatic moiety (cycloalkyl, cycloalkenyl or aromatic) group of six or less carbon atoms for every ten carbon atoms in the substituent. Usually, however, the substituents contain no more than one such non-aliphatic group for every fifty carbon atoms, and in many cases, they contain no such non-aliphatic groups at all; that is, the typical substituents are purely aliphatic. Typically, these purely aliphatic substituents are alkyl or alkenyl groups.

Specific examples of the substantially saturated hydrocarbon-based substituents containing an average of more than 30 carbon atoms are the following: a mixture of poly(ethylene/propylene) groups of 35 to 70 carbon atoms, a mixture of oxidatively or mechanically degraded poly(ethylene/propylene) groups of 35 to 70 carbon atoms, a mixture of poly(proplene/1-hexene) groups of 80 to 150 carbon atoms, and a mixture of polyisobutene groups having an average of 50 to 75 carbon atoms.

A preferred source of the substituents are polyisobutenes obtained by polymerisation of a C₄ refinery stream having a butene content of 35 to 75 weight per cent and isobutene content of 30 to 60 weight per cent in the presence of a Lewis acid catalyst such as aluminium trichloride or boron trifluoride. These polyisobutenes contain predominantly (greater than 80% of total repeating units) isobutene repeating units of the configuration:

-C(CH₃)₂CH₂-

Exemplary of amino compounds useful in making these acylated compounds are the following:
(1) polyalkylene polyamines of the general formula:

   (R⁴)₂N[P-N(R⁴)]ₘR⁴ (IV)

   wherein each R⁴ is independently a hydrogen atom, a hydrocarbyl group or a hydroxy-substituted hydrocarbyl group containing up to 30 carbon atoms, with the proviso that at least one R⁴ is a hydrogen atom, m is a whole number of 1 to 10 and P is a C₁₋₁₈ alkylene group;
(2) hydroxyalkyl-substituted polyamines wherein the polyamines are as described above;
(3) heterocyclic-substituted polyamines wherein the polyamines are as described above and the heterocyclic substituent is derived from, for example, piperazine, imidazoline, pyrimidine or morpholine; and
(4) aromatic polyamines of the general formula:

   Ar(NR⁴ ₂)_{z} (V)

   wherein Ar is an aromatic nucleus of 6 to 20 carbon atoms, each R⁴ is as defined above and z is 2 to 8.

Specific examples of polyalkylene polyamines of formula IV are ethylene diamine, tetra(ethylene)pentamine, tri-(trimethylene)tetramine and 1,2-propylene diamine.

Specific examples of hydroxyalkyl-substituted polyamines include N-(2-hydroxyethyl) ethylene diamine, N,N'-bis-(2-hydroxyethyl) ethylene diamine and N-(3-hydroxybutyl) tetramethylene diamine.

Specific examples of heterocyclic-substituted polyamines are N-2-aminoethyl piperazine, N-2- and N-3-amino propyl morpholine, N-3-(dimethyl amino) propyl piperazine, 2-heptyl-3-(2-aminopropyl) imidazoline, 1,4-bis (2-aminoethyl) piperazine, 1-(2-hydroxy ethyl) piperazine, and 2-heptadecyl-1-(2-hydroxyethyl)-imidazoline.

Specific examples of aromatic polyamines are the various isomeric phenylene diamines and the various isomeric naphthalene diamines.

Many patents have described useful acylated nitrogen compounds including U.S. Patents Nos. 3,172,892, 3,219,666, 3,272,746, 3,310,492, 3,341,542, 3,444,170, 3,455,831, 3,455,832, 3,576,743, 3,630,904, 3,632,511, 3,804,763 and 4,234,435. A typical acylated nitrogen-containing compound of this class is that made by reacting a polyisobutene-substituted succinic anhydride acylating agent wherein the polyisobutene substituent has from 50 to 400 carbon atoms with a mixture of ethylene polyamines having 3 to 7 amino nitrogen atoms per ethylene polyamine.

Another type of acylated nitrogen compound belonging to this class is that made by reacting the aforementioned alkylene amines with the aforementioned substituted succinic acids or anhydrides and aliphatic monocarboxylic acids having from 2 to 22 carbon atoms. In these types of acylated nitrogen compounds, the mole ratio of succinic acid to monocarboxylic acid is in the range from 1:0.1 to 1:1. Typical of the monocarboxylic acid are formic acid, acetic acid, dodecanoic acid, butanoic acid, oleic acid, stearic acid, the commercial mixture of stearic acid isomers known as isostearic acid and tolyl acid. Such materials are more fully described in U.S. Patents Nos. 3,216,936 and 3,250,715.

Still another type of acylated nitrogen compound useful in the gasoline compositions of the invention is the product of the reaction of a fatty monocarboxylic acid of 12 to 30 carbon atoms and the aforementioned alkylene amines, typically, ethylene, propylene or trimethylene polyamines containing 2 to 8 amino groups and mixtures thereof. The fatty monocarboxylic acids are generally mixtures of straight and branched chain fatty carboxylic acids containing 12 to 30 carbon atoms. A widely used type of acylated nitrogen compound is made by reacting the aforementioned alkylene polyamines with a mixture of fatty acids having from 5 to 30 mole per cent straight chain acid and 70 to 95 mole per cent branched chain fatty acids. Among the commercially available mixtures are those known widely in the trade as isostearic acid. These mixtures are produced as a by-product from the dimerisation of unsaturated fatty acids as described in U.S. Patents Nos. 2,812,342 and 3,260,671.

The branched chain fatty acids can also include those in which the branch is not alkyl in nature, such as found in phenyl and cyclohexyl stearic acid and the chloro-stearic acids. Branched chain fatty carboxylic acid/alkylene polyamine products have been described, for example in U.S. Patents Nos. 3,110,673, 3,251,853, 3,326,801, 3,337,459, 3,405,064, 3,429,674, 3,468,639 and 3,857,791.

The phenol/aldehyde/amino compound condensates useful as dispersants in the gasoline compositions of the invention include those generically referred to as Mannich condensates. Generally, they are made by reacting simultaneously or sequentially at least one active hydrogen compound such as a hydrocarbon-substituted phenol (e.g., an alkyl phenol wherein the alkyl group has at least an average of 12 to 400, preferably 30 to 400, carbon atoms), having at least one hydrogen atom bonded to an aromatic carbon, with at least one aldehyde or aldehyde-producing material (typically formaldehyde precursor) and at least one amino or polyamino compound having at least one NH group. The amino compounds include primary or secondary monoamines having hydrocarbon substituents of 1 to 30 carbon atoms or hydroxyl-substituted hydrocarbon substituents of 1 to 30 carbon atoms. Another type of typical amino compound are the polyamines described during the discussion of the acylated nitrogen-containing compounds.

Exemplary monoamines include methyl etheyl amine, methyl octadecyl amines, aniline, diethyl amine, diethanoi amine and dipropyl amine. The following patents contain extensive descriptions of Mannich condensates: U.S. Patents Nos. 2,459,112, 3,413,347, 3,558,743, 2,962,442, 3,442,808, 3,586,629, 2,984,550, 3,448,047, 3,591,598, 3,036,003, 3,454,497, 3,600,372, 3,166,516, 3,459,661, 3,634,515, 3,236,770, 3,461,172, 3,649,229, 3,355,270, 3,493,520, 3,697,574, 3,368,972 and 3,539,633.

Condensates made from sulphur-containing reactants can also be used in the gasoline compositions of the present invention. Such sulphur-containing condensates are described in U.S. Patents Nos. 3,368,972, 3,649,229, 3,600,372, 3,649,659 and 3,741,896. These patents also disclose sulphur-containing Mannich condensates. Generally the condensates used in making compositions of this invention are made from a phenol bearing an alkyl substituent of 6 to 400 carbon atoms, more typically, 30 to 250 carbon atoms. These typical condensates are made from formaldehyde or C₂₋₇ aliphatic aldehyde and an amino compound such as those used in making the acylated nitrogen-containing compounds described above.

These preferred condensates are prepared by reacting one molar portion of phenolic compound with 1 to 2 molar portions of aldehyde and 1 to 5 equivalent portions of amino compound (an equivalent of amino compound is its molecular weight divided by the number of -NH groups present). The conditions under which such condensation reactions are carried out are well known to those skilled in the art.

A particularly preferred class of nitrogen-containing condensation products for use in the gasoline compositions of the present invention are those made by (1) reacting at least one hydroxy aromatic compound containing an aliphatic-based or cycloaliphatic-based substituent which has at least 30 carbon atoms and up to 400 carbon atoms with a lower aliphatic C₁₋₇ aldehyde or reversible polymer thereof in the presence of an alkaline reagent, such as an alkali metal hydroxide, at a temperature up to 150°c; (2) substantially neutralising the intermediate reaction mixture thus formed; and (3) reacting the neutralised intermediate with at least one compound which contains an amino group having at least one -NH- group.

More preferably, these condensates are made from (a) phenols bearing a hydrocarbon-based substituent having 30 to 250 carbon atoms, said substituent being derived from a polymer of propylene, 1-butene, 2-butene, or isobutene and (b) formaldehyde, or reversible polymer thereof, (e.g., trioxane, paraformaldehyde) or functional equivalent thereof, (e.g., methylol) and (c) an alkylene polyamine such as ethylene polyamines having from 2 to 10 nitrogen atoms.

The esters useful as dispersants in the gasoline compositions of the invention are derivatives of substituted carboxylic acids in which the substituent is a substantially aliphatic, substantially saturated hydrocarbon-based group containing at least 30, preferably at least 50, up to 750 aliphatic carbon atoms. As used herein, the term "hydrocarbon-based group" denotes a group having a carbon atom directly attached to the remainder of the molecule and having predominantly hydrocarbon character within the context of this invention. Such groups include the following:
(1) Hydrocarbon groups; that is, aliphatic groups, aromatic-andalicyclic-substituted aliphatic groups, and the like, of the type known to those skilled in the art.
(2) Substituted hydrocarbon groups; that is, groups containing non-hydrocarbon substituents which, in the context of this invention, do not alter the predominantly hydrocarbon character of the group. Those skilled in the art will be aware of suitable substituents; examples are halo, nitro, hydroxy, alkoxy, carbalkoxy and alkylthio.
(3) Hetero groups; that is, groups which, while predominantly hydrocarbon in character within the context of this invention, contain atoms other than carbon present in a chain or ring otherwise composed of carbon atoms. Suitable hetero atoms will be apparent to those skilled in the art and include, for example, nitrogen, oxygen and sulphur.

In general, no more than about three substituents or hetero atoms, and preferably no more than one, will be present for each 10 carbon atoms in the hydrocarbon-based group.

The substituted carboxylic acids are normally prepared by the alkylation of an unsaturated acid, or a derivative thereof such as an anhydride, with a source of the desired hydrocarbon-based group. Suitable unsaturated acids and derivatives thereof include acrylic acid, methacrylic acid, maleic acid, maleic anhydride, fumaric acid, itaconic acid, itaconic anhydride, citraconic acid, citraconic anhydride, mesaconic acid, glutaconic acid, chloromaleic acid, aconitic acid, crotonic acid, methylcrotonic acid, sorbic acid, 3-hexenoic acid, 10-decenoic acid and 2-pentene-1,3,5-tricarboxylic acid. Particularly preferred are the unsaturated dicarboxylic acids and their derivatives, especially maleic acid, fumaric acid and maleic anhydride.

Suitable alkylating agents include homopolymers and interpolymers of polymerisable olefin monomers containing from 2 to 10 and usually from 2 to 6 carbon atoms, and polar substituent-containing derivatives thereof. Such polymers are substantially saturated (i.e., they contain no more than about 5% olefinic linkages) and substantially aliphatic (i.e., they contain at least 80% and preferably at least 95% by weight of units derived from aliphatic monoolefins). Illustrative monomers which may be used to produce such polymers are ethylene, propylene, 1-butene, 2-butene, isobutene, 1-octene and 1-decene. Any unsaturated units may be derived from conjugated dienes such as 1,3-butadiene and isoprene; non-conjugated dienes such as 1,4-hexadiene, 1,4-cyclohexadiene, 5-ethylidene-2-norbornene and 1,6-octadiene; and trienes such as 1-isopropylidene-3a,4,7,7a.tetrahydroindene, 1-isopropylidenedicyclopentadiene and 2-(2-methylene-4-methyl-3-pentenyl)[2,2,1]bicyclo-5-heptene.

A first preferred class of polymers comprises those of terminal olefins such as propylene, 1-butene, isobutene and 1-hexene. Especially preferred within this class are polybutenes comprising predominantly isobutene units. A second preferred class comprises terpolymers of ethylene, a C₃₋₈ alpha-monoolefin and a polyene selected from the group consisting of non-conjugated dienes (which are especially preferred) and trienes. Illustrative of these terpolymers is "Ortholeum 2052" manufactured by E.I. duPont de Nemours & Company, which is a terpolymer containing about 48 mole per cent ethylene groups, 48 mole per cent propylene groups and 4 mole per cent 1,4-hexadiene groups and having an inherent viscosity of 1.35 (8.2 grams of polymer in 10 ml of carbon tetrachloride at 30°C).

Methods for the preparation of the substituted carboxylic acids and derivatives thereof are well known in the art and need not be described in detail. Reference is made, for example, to U.S. Patents Nos. 3,272,746, 3,522,179 and 4,234,435. The mole ratio of the polymer to the unsaturated acid or derivative thereof may be equal to, greater than or less than 1, depending on the type of product desired.

The esters are those of the above-described substituted carboxylic acids with hydroxy compounds which may be aliphatic compounds such as monohydric and polyhydric alcohols or aromatic compounds such as phenols and naphthols. Examples of aromatic hydroxy compounds include phenol, beta-naphthol, alpha-naphthol, cresol, resorcinol, catechol, p,p'-dihydroxybiphenyl, 2-chlorophenol, 2,4-dibutylphenol, propene tetramer-substituted phenol, didodecylphenol, 4,4' -methylene-bis-phenol, alpha-decyl-beta-naphthol, polyisobutene (molecular weight of 1000)-substituted phenol, the condensation product of heptylphenol with formaldehyde, the condensation product of octyl-phenol with acetone, di(hydroxyphenyl)-oxide, di(hydroxyphenyl)sulphide, di(hydroxyphenyl)disulphide, and 4-cyclo-hexylphenol. Phenol and alkylated phenols having up to three alkyl substituents are preferred. Each of the alkyl substituents may contain 100 or more carbon atoms.

The aliphatic alcohols from which the esters may be derived preferably contain up to 40 aliphatic carbon atoms. They may be monohydric alcohols such as methanol, ethanol, isooctanol, dodecanol, cyclohexanol, cyclopentanol, behenyl alcohol, hexatriacontanol, neopentyl alcohol, isobutyl alcohol, benzyl alcohol, beta-phenylethyl alcohol, 2-methylcyclohexanol, beta-chloroethanol, monomethyl ether of ethylene glycol, monobutyl ether of ethylene glycol, monopropyl ether of diethylene glycol, monododecyl ether of triethylene glycol, monooleate of ethylene glycol, monostearate of diethylene glycol, secpentyl alcohol, tertbutyl alcohol, 5-bromo-dodecanol, nitro-octadecanol and dioleate of glycerol. The polyhydric alcohols preferably contain from 2 to 10 hydroxy radicals. They are illustrated by, for example, ethylene glycol, diethylene glycol, triethylene glycol, tetraethylene glycol, dipropylene glycol, tripropylene glycol, dibutylene glycol, tri-butylene glycol, and other alkylene glycols in which the alkylene radical contains from 2 to 8 carbon atoms. Other useful polyhydric alcohols include glycerol, monooleate of glycerol, monostearate of glycerol, monomethyl ether of glycerol, pentaerythritol, 9,10-dihydroxy stearic acid, methyl ester of 9,10-dihydroxy stearic acid, 1,2-butanediol, 2,3-hexanediol, 2,4-hexanediol, penacol, erythritol, arabitol, sorbitol, mannitol, 1,2-cyclohexanediol, and xylene glycol. Carbohydrates such as sugars, starches and cellulose may also yield esters useful in this invention. The carbohydrates may be exemplified by glucose, fructose, sucrose, rhamnose, mannose, glyceraldehyde and galactose.

An especially preferred class of polyhydric alcohols are those having at least three hydroxy radicals, some of which have been esterified with a monocarboxylic acid having from 8 to 30 carbon atoms, such as octanoic acid, oleic acid, stearic acid, linoleic acid, dodecanoic acid, or tall oil acid. Examples of such partially esterified polyhydric alcohols are the monooleate of sorbitol, distearate of sorbitol, monooleate of glycerol, monostearate of glycerol, di-dodecanoate of erythritol.

The esters may also be derived from unsaturated alcohols such as allyl alcohol, cinnamyl alcohol, propargyl alcohol, 1-cyclohexene-3-ol and oleyl alcohol. Still another class of the alcohols capable of yielding the esters useful in this invention comprise the ether-alcohols and amino-alcohols including, for example, the oxyalkylene-, oxyarylene-, amino-alkylene- and amino-arylene-substituted alcohols having one or more oxyalkylene, oxyarylene, amino-alkylene or amino-arylene radicals. They are exemplified by Cellosolve, carbitol, phenoxyethanol, heptylphenyl- (oxypropylene)₆-H, octyl-(oxyethylene)₃₀-H, phenyl-(oxyoctylene)₂-H, mono(heptylphenyl-oxypropylene)substituted glycerol, poly(styrene oxide), amino-ethanol, 3-amino ethyl-pentanol, di(hydroxyethyl) amine, p-amino-phenol, tri(hydroxypropyl)amine, N-hydroxyethyl ethylene diamine and N,N,N',N'-tetrahydroxy-trimethylene diamine. For the most part, the ether-alcohols having up to about 150 oxyalkylene radicals in which the alkylene radical contains from 1 to 8 carbon atoms are preferred.

The esters may be diesters of succinic acids or acidic esters, i.e., partially esterified polyhydric alcohols or phenols, i.e., esters having free alcoholic or phenolic hydroxyl radicals. Mixtures of the above-illustrated esters likewise are contemplated within the scope of the invention.

The succinic acid esters may be prepared by one of several methods. The method which is preferred because of convenience and superior properties of the esters it produces, involves the reaction of a suitable alcohol or phenol with a substantially hydrocarbon-substituted succinic anhydride. The esterification is usually carried out at a temperature above about 100°C, preferably between 150°C and 300°C.

The water formed as a by-product is removed by distillation as the esterification proceeds. A solvent may be used in the esterification to facilitate mixing and temperature control. It also facilitates the removal of water from the reaction mixture. The useful solvents include xylene, toluene, diphenyl ether, chlorobenzene and mineral oil.

A modification of the above process involves the replacement of the substituted succinic anhydride with the corresponding succinic acid. However, succinic acids readily undergo dehydration at temperatures above about 100°C and are thus converted to their anhydrides which are then esterified by the reaction with the alcohol reactant. In this regard, succinic acids appear to be the substantial equivalent of their anhydrides in the process.

The relative proportions of the succinic reactant and the hydroxy reactant which are to be used depend to a large measure upon the type of the product desired and the number of hydroxyl groups present in the molecule of the hydroxy reactant. For instance, the formation of a half ester of a succinic acid, i.e., one in which only one of the two acid radicals is esterified, involves the use of one mole of a monohydric alcohol for each mole of the substituted succinic acid reactant, whereas the formation of a diester of a succinic acid involves the use of two moles of the alcohol for each mole of the acid. On the other hand, one mole of a hexahydric alcohol may combine with as many as six moles of a succinic acid to form an ester in which each of the six hydroxyl radicals of the alcohol is esterified with one of the two acid radicals of the succinic acid. Thus, the maximum proportion of the succinic acid to be used with a polyhydric alcohol is determined by the number of hydroxyl groups present in the molecule of the hydroxy reactant. For the purposes of this invention, it has been found that esters obtained by the reaction of equimolar amounts of the succinic acid reactant and hydroxy reactant have superior properties and are therefore preferred.

In some instances, it is advantageous to carry out the esterification in the presence of a catalyst such as sulphuric acid, pyridine hydrochloride, hydrochloric acid, benzenesulphonic acid, p-toluenesulphonic acid, phosphoric acid, or any other known esterification catalyst. The amount of the catalyst in the reaction may be as little as 0.01% (by weight of the reaction mixture), more often from 0.1% to 5%.

The succinic acid esters may alternatively be obtained by the reaction of a substituted succinic acid or anhydride with an epoxide or a mixture of an epoxide and water. Such reaction is similar to one involving the acid or anhydride with a glycol. For instance, the product may be prepared by the reaction of a substituted succinic acid with one mole of ethylene oxide. Similarly, the product may be obtained by the reaction of a substituted succinic acid with two moles of ethylene oxide. Other epoxides which are commonly available for use in such reaction include, for example, propylene oxide, styrene oxide, 1,2-butylene oxide, 2,3-butylene oxide, epichlorohydrin, cyclohexene oxide, 1,2-octylene oxide, epoxidised soya bean oil, methyl ester of 9,10-epoxy-stearic acid and butadiene mono-epoxide. For the most part, the epoxides are the alkylene oxides in which the alkylene radical has from 2 to 8 carbon atoms; or the epoxidised fatty acid esters in which the fatty acid radical has up to 30 carbon atoms and the ester radical is derived from a lower alcohol having up to 8 carbon atoms.

In lieu of the succinic acid or anhydride, a lactone acid or a substituted succinic acid halide may be used in the processes illustrated above. Such acid halides may be acid dibromides, acid dichlorides, acid monochlorides, and acid monobromides. The substituted succinic anhydrides and acids can be prepared by, for example, the reaction of maleic anhydride with a high molecular weight olefin or a halogenated hydrocarbon such as is obtained by the chlorination of an olefin polymer described previously. The reaction involves merely heating the reactants at a temperature preferably from 100°C to 250°C. The product from such a reaction is an alkenyl succinic anhydride. The alkenyl group may be hydrogenated to an alkyl group. The anhydride may be hydrolysed by treatment with water or steam to the corresponding acid. Another method useful for preparing the succinic acids or anhydrides involves the reaction of itaconic acid or anhydride with an olefin or a chlorinated hydrocarbon at a temperature usually within the range from 100°C to 250°C. The succinic acid halides can be prepared by the reaction of the acids or their anhydrides with a halogenation agent such as phosphorous tribromide, phosphorus pentachloride, or thionyl chloride. These and other methods of preparing the succinic compounds are well known in the art and need not be illustrated in further detail here.

Still further methods of preparing esters useful in the gasoline compositions of the present invention are available. For instance, the esters may be obtained by the reaction of maleic acid or anhydride with an alcohol such as is illustrated above to form a mono- or di-ester of maleic acid and then the reaction of this ester with an olefin or a chlorinated hydrocarbon such as is illustrated above. They may also be obtained by first esterifying itaconic anhydride or acid and subsequently reacting the ester intermediate with an olefin or a chlorinated hydrocarbon under conditions similar to those described hereinabove.

A large number of different types of polymeric dispersants have been suggested as useful in lubricating oil formulations, and such polymeric dispersants are useful in the gasoline compositions of the present invention. Often, such additives have been described as being useful in lubricating formulations as viscosity index improvers with dispersing characteristics. The polymeric dispersants generally are polymers or copolymers having a long carbon chain and containing "polar" groups to impart the dispersancy characteristics. Examples of polar groups include amino, amido, imino, imido, hydroxyl and ether groups. For example, the polymeric dispersants may be copolymers of methacrylates or acrylates containing additional polar groups, ethylene/propylene copolymers containing polar groups or vinyl acetate/fumaric acid ester copolymers.

Many such polymeric dispersants have been described in the prior art, for example in U.S. Patents Nos. 4,402,844, 3,356,763 and 3,891,721.

A number of the polymeric dispersants may be prepared by grafting polar monomers on to polyolefinic backbones. For example, U.S. Patent Nos. 3,687,849 and 3,687,905 describe the use of maleic anhydride as a graft monomer to a polyolefinic backbone. Maleic acid or anhydride is particularly desirable as a graft monomer because this monomer is relatively inexpensive, provides an economical route to the incorporation of dispersant nitrogen compounds into polymers by further reaction of the carboxyl groups of the maleic acid or anhydride with, for example, nitrogen compounds or hydroxy compounds. U.S. Patent No. 4,160,739 describes graft copolymers obtained by the grafting of a monomer system comprising maleic acid or anhydride and at least one other different monomer which is addition copolymerisable therewith, the grafted monomer system then being post-reacted with a polyamine. The monomers which are copolymerisable with maleic acid or anhydride are any alpha, beta-monoethylenically unsaturated monomers which are sufficiently soluble in the reaction medium and reactive towards maleic acid or anhydride so that substantially larger amounts of maleic acid or anhydride can be incorporated into the grafted polymeric product. Accordingly, suitable monomers include the esters, amides and nitriles of acrylic and methacrylic acid, and monomers containing no free acid groups. The incorporation of heterocyclic monomers into graft polymers is described by a process which comprises a first step of graft polymerising an alkyl ester of acrylic acid or methacrylic acid, alone or in combination with styrene, onto a backbone copolymer which is a hydrogenated block copolymer of styrene and a conjugated diene having 4 to 6 carbon atoms to form a first graft polymer. In the second step, a polymerisable heterocyclic monomer, alone or in combination with a hydrophobising vinyl ester is co-polymerised onto the first graft copolymer to form a second graft copolymer.

Other patents describing graft polymers useful as dispersants in the gasoline compositions of this invention include U.S. Patents Nos. 3,243,481, 3,475,514, 3,723,575, 4,026,167, 4,085,055, 4,181,618 and 4,476,283.

Another class of polymeric dispersant useful in the gasoline compositions of the invention are the so-called "star" polymers and copolymers. Such polymers are described in, for example U.S. Patents Nos. 4,346,193, 4,141,847, 4,358,565, 4,409,120 and 4,077,893.

The hydrocarbon-substituted phenolic dispersants useful in the gasoline compositions of the present invention include the hydrocarbon-substituted phenolic compounds wherein the hydrocarbon substituents have a molecular weight which is sufficient to render the phenolic compound fuel soluble. Generally, the hydrocarbon substituent will be a substantially saturated, hydrocarbon-based group of at least 30 carbon atoms. The phenolic compounds may be represented generally by the following formula:

(R⁵)ₑ-Ar¹-(OH)_{f} (VI)

wherein R⁵ is a substantially saturated hydrocarbon-based substituent having an average of from 30 to 400 aliphatic carbon atoms, and e and f are each 1, 2 or 3. Ar¹ is an aromatic moiety such as a benzene nucleus, naphthalene nucleus or linked benzene nuclei. Optionally, the above phenates as represented by formula VI may contain other substituents such as lower alkyl, lower alkoxy, nitro, amino and halo groups. Preferred examples of optional substituents are the nitro and amino groups.

The substantially saturated hydrocarbon-based group R⁵ in formula VI may contain up to 750 aliphatic carbon atoms although it usually has a maximum of an average of 400 carbon atoms. In some instances R⁵ has a minimum of 50 carbon atoms. As noted, the phenolic compounds may contain more than one R⁵ group for each aromatic nucleus in the aromatic moiety Ar¹.

Generally, the hydrocarbon-based groups R⁵ are derived from homo- or interpolymers (e.g., copolymers, terpolymers) of mono- and diolefins having 2 to 10 carbon atoms, such as ethylene, propylene, butene-1, isobutene, butadiene, isoprene, 1-hexene and 1-octene. Typically, these olefins are 1-monoolefins. The R⁵ groups can also be derived from the halogenated (e.g., chlorinated or brominated) analogues of such homo- or interpolymers. The R⁵ groups can, however, be made from other sources, such as monomeric high molecular weight alkenes (e.g. 1-tetracontene) and chlorinated analogues and hydrochlorinated analogues thereof, aliphatic petroleum fractions, particularly paraffin waxes and cracked and chlorinated analogues and hydrochlorinated analogues thereof, white oils, synthetic alkenes such as those produced by the Ziegler-Natta process (e.g., poly(ethylene) greases) and other sources known to those skilled in the art. Any unsaturation in the R⁵ groups may be reduced or eliminated by hydrogenation according to procedures known in the art before the nitration step described hereafter.

Specific examples of the substantially saturated hydrocarbon-based R⁵ groups are the following: a tetracontanyl group, a henpentacontanyl group, a mixture of poly(ethylene/propylene) groups of 35 to 70 carbon atoms, a mixture of oxidatively or mechanically degraded poly(ethylene/propylene) groups of 35 to 70 carbon atoms, a mixture of poly(propylene/1-hexene) groups of 80 to 150 carbon atoms, a mixture of polyisobutene groups having 20 to 32 carbon atoms, and a mixture of polyisobutene groups having an average of 50 to 75 carbon atoms.

A preferred source of the group R⁵ are polyisobutenes obtained by polymerisation of a C₄ refinery stream having a butene content of 35 to 75 weight per cent and isobutene content of 30 to 60 weight per cent in the presence of a Lewis acid catalyst such as aluminium trichloride or boron trifluoride. These polyisobutenes contain predominatly (greater than 80% of total repeat units) isobutene repeating units of the configuration.

-C(CH₃)₂CH₂-

The attachment of the hydrocarbon-based group R⁵ to the aromatic moiety Ar¹ can be accomplished by a number of techniques well known to those skilled in the art.

In one preferred embodiment, the phenolic dispersants useful in the gasoline compositions of the present invention are hydrocarbon-substituted nitro phenols as represented by formula VI wherein the optional substituent is one or more nitro groups. The nitro phenols can be conveniently prepared by nitrating appropriate phenols, and typically, the nitro phenols are formed by nitration of alkyl phenols having an alkyl group of at least 30 and preferably at least 50 carbon atoms. The preparation of a number of hydrocarbon-substituted nitro phenols useful in the gasoline compositions of the present invention is described in U.S. Patent No. 4,347,148.

In another preferred embodiment, the hydrocarbon-substituted phenol dispersants useful in the present invention are hydrocarbon-substituted amino phenols such as represented by formula VI wherein the optional substituent is one or more amino groups. These amino phenols can conveniently be prepared by nitrating an appropriate hydroxy aromatic compound as described above and thereafter reducing the nitro groups to amino groups. Typically, the useful amino phenols are formed by nitration and reduction of alkyl phenols having an alkyl or alkenyl group of at least 30 and preferably at least 50 carbon atoms. The preparation of a large number of hydrocarbon-substituted amino phenols useful as dispersants in the present invention is described in U.S. Patent No. 4,320,021.

Also useful as dispersants in the gasoline compositions of the present invention are fuel-soluble alkoxylated derivatives of alcohols, phenols and amines. A wide variety of such derivatives can be utilised as long as the derivatives are fuel-soluble. More preferably, the derivatives in addition to being fuel-soluble should be water-insoluble. Accordingly, in a preferred embodiment, the fuel-soluble alkoxylated derivatives useful as the dispersants are characterised as having an HLB of from 1 to 13.

As is well known to those skilled in the art, the fuel-solubility and water-insolubility characteristics of the alkoxylated derivatives can be controlled by selection of the alcohol, phenol or amine, selection of the particular alkoxy reactant, and by selection of the amount of alkoxy reactant which is reacted with the alcohol, phenol or amine. Accordingly, the alcohols which are utilised to prepare the alkoxylated derivatives are hydrocarbon- based alcohols while the amines are hydrocarbyl-substituted amines as described above. The phenols may be phenols or hydrocarbon-substituted phenols and the hydrocarbon substituent may contain as few as 1 carbon atom.

The alkoxylated derivatives are obtained by reacting the alcohol, phenol or amine with an epoxide or a mixture of an epoxide and water. For example, the derivative may be prepared by the reaction of the alcohol, phenol or amine with an equal molar amount or an excess of ethylene oxide. Other epoxides which can be reacted with the alcohol, phenol or amine include, for example, propylene oxide, styrene oxide, 1,2-butylene oxide, 2,3-butylene oxide, epichlorohydrin, cyclohexene oxide and 1,2-octylene oxide. Preferably, the epoxides are the alkylene oxides in which the alkylene group has from 2 to 8 carbon atoms. As mentioned above, it is desirable and preferred that the amount of alkylene oxide reacted with the alcohol, phenol or amine be insufficient to render the derivative water-soluble.

The following are examples of commercially available alkylene oxide derivatives which may be utilised as dispersants in the gasoline compositions of the present invention: Ethomeen S/12, tertiary amines ethylene oxide condensation products of the primary fatty amines (HLB, 4.15; Armak Industries); and Plurafac A-24, an oxyethylated straight-chain alcohol available from BASF Wyandotte Industries (HLB 5.0). Other suitable fuel-soluble alkoxylated derivatives of alcohols, phenols and amines will be readily apparent to those skilled in the art.

In a particularly preferred embodiment, further to the polyalphaolefin and the polyoxyalkylene compound, the gasoline composition of the invention may additionally contain, as ashless dispersant, a minor amount of a polyolefin-substituted succinimide derivative wherein the polyolefin has Mₙ in the range 800 to 5000, preferably 1000 to 5000, more preferably at least 1750, 1800 or 1850 and at most 4000, 3500, 3000 or 2500. The amine from which the succinimide is formed is preferably a C₁₋₃₀ amine, especially a C₄₋₁₂ amine containing 3 to 7 nitrogen atoms, e.g. diethylene triamine, triethylene tetramine, tetramethylene pentamine, pentaethylene hexamine, hexaethylene heptamine, tripropylene tetramine and mixtures of any 2 or more thereof.

Preferably the hydrocarbon-soluble ashless dispersant is present in an amount in the range 30 to 500 ppmw, more preferably 100 to 300 ppmw, based on total composition.

The gasoline composition may additionally include (e.g. as an alternative to inclusion of succinimide derivative) an oil soluble polyamine as described in EP-A-290 088 or an N-substituted carbamate as described in EP-A-414 963, in each case in similar quantities to those described therein.

The gasoline composition may further include, as flame-speed improver, an alkali metal or alkaline earth metal salt of a succinic acid derivative as described in EP-A-290 088, in similar quantities to those described therein.

Apart from components already described above, the gasoline composition may also contain other additives. Thus, it can contain a lead compound as anti-knock additive, and accordingly the gasoline composition according to the invention includes both leaded and unleaded gasoline. The gasoline composition can also contain antioxidants such as phenolics, e.g. 2,6-di-tert-butyl-phenol, or phenylenediamines, e.g. N,N -di-sec-butyl-p-phenylene-diamine, or antiknock additives other than lead compounds, or polyether amino additives, e.g. as described in US Patent No. 4,477,261 and EP-A-151 621.

The gasoline composition according to the invention comprises a major amount of a gasoline (base fuel) suitable for use in spark-ignition engines. This includes hydrocarbon base fuels boiling essentially in the gasoline boiling range from 30 to 230°c. These base fuels may comprise mixtures of saturated, olefinic and aromatic hydrocarbons. They can be derived from straight-run gasoline, synthetically produced aromatic hydrocarbon mixtures, thermally or catalytically cracked hydrocarbon feedstocks, hydrocracked petroleum fractions or catalytically reformed hydrocarbons. The octane number of the base fuel is not critical and will generally be above 65. In the gasoline, hydrocarbons can be replaced up to substantial amounts by alcohols, ethers, ketones, or esters. Naturally, the base fuels are desirably substantially free of water, since water may impede a smooth combustion.

The polyalphaolefin and polyoxyalkylene compound may conveniently be added as a blend with other chosen additives. A convenient method for preparing the gasoline composition is therefore to prepare a concentrate of the polyalphaolefin and polyoxyalkylene compound together with the other additives, and then to add this concentrate to the gasoline in the amount required to produce the required final concentrations of additives.

The invention accordingly further provides a concentrate suitable for addition to gasoline which comprises a gasoline-compatible diluent, a polyalphaolefin as defined above, a polyoxyalkylene compound as defined above, the weight ratio polyalphaolefin:polyoxyalkylene compound being in the range 1:10 to 10:1, and optionally also at least one hydrocarbon-soluble ashless dispersant.

Advantageously, the polyalphaolefin and the polyoxyalkylene compound together are present in an amount in the range 20% to 80% w and the ashless dispersant, if present, is present in an amount in the range 5% to 30% w, all percentages being calculated on the diluent.

Suitable gasoline-compatible diluents include hydrocarbons, e.g. heptane, alcohols or ethers, such as methanol, ethanol, propanol, 2-butoxyethanol or methyl tert-butyl ether. Preferably the diluent is an aromatic hydrocarbon solvent such as toluene, xylene, mixtures thereof or mixtures of toluene or xylene with an alcohol. The solvent is preferably toluene. Optionally, the concentrate may contain a dehazer, particularly a polyether-type ethoxylated alkylphenol-formaldehyde resin. The dehazer, if employed, can suitably be present in the concentrate in an amount of from 0.01 to 2%w, calculated on the diluent.

In a further aspect, the invention provides a method for operating a spark-ignition internal combustion engine which comprises introducing into the combustion chambers of said engine a gasoline composition as defined above in accordance with the invention.

The invention will be further understood from the following illustrative examples. In the examples, various additives are designated as follows:-
(a) "PGHE" is a polyoxypropylene glycol hemiether (monoether) prepared using a mixture of C₁₂₋₁₅ alcohols as initiator, and having Mₙ in the range 1200 to 1500 and a kinematic viscosity in the range 72 to 82 mm²/s at 40°C according to ASTM D 445, available under the trade designation "SAP 949" from member companies of the Royal Dutch/Shell group;
(b) "PAO" is a polyalphaolefin, being a hydrogenated oligomer of decene-1 having a viscosity at 100°C of 8 x 10⁻⁶ m²/s (8 centistokes).
(c) "PMP" is a 40% w/w solution in xylene of polyisobutylene succinimide prepared by reaction of a polyisobutylene of number average molecular weight (Mₙ) 2470 (determined by quantitative reaction with ozone) with maleic anhydride, followed by reaction of the resulting polyisobutylene succinic anhydride product with a mixture of tetraethylene pentamine, pentaethylene hexamine and hexamethylene heptamine (molar ratio 1:2:1) in molar ratio anhydride:amine of 2:1.

In the examples which follow, amounts of PMP are quoted as amounts of solution, and where amounts of xylene are quoted, these do not include the xylene associated in the 40% w/w solutions of PMP.

In the examples, additive concentrates were prepared by taking samples of PMP and adding, with stirring at 20°C, amounts of PAO (and additional xylene), followed by addition of amounts of PGHE. Samples of these additive concentrates were then incorporated into gasoline compositions, with stirring, in amounts to give desired concentrations of components. This mirrors actual industry practice, and it is important both for the additive concentrates to be fully stable, and for gasolines containing the additives to give good performance in terms of engine cleanliness and avoidance of valve sticking.

### EXAMPLES 1 to 8

Additive concentrates in accordance with the invention and comparative examples were prepared as described above and stored for 6 weeks at 20°C and -20°C, after which stability was assessed visually. Results are given in Table I.

**TABLE I**

| Example | Quantities (g) | | | | Ratio PHGE: PAO | Storage (6 weeks) at 20°C and -20°C |
|---|---|---|---|---|---|---|
| | PMP | Additive Oil | | Additional Xylene | | |
| | | PHGE | PAO | | | |
| Comp. A | 20 | 25 | - | 105 | 1:0 | deposits |
| 1 | 20 | 12.5 | 12.5 | 40 | 1:1 | clear |
| | | | | | | |
| Comp. B | 30 | 30 | - | 100 | 1:0 | slightly hazy ⁺ |
| 2 | 30 | 15 | 15 | 40 | 1:1 | clear |
| | | | | | | |
| Comp. C | 30 | 40 | - | 90 | 1:0 | phase separation ⁺ |
| 3 | 30 | 20 | 20 | 60 | 1:1 | clear |
| 4 | 30 | 25 | 15 | 80 | 1.67:1 | clear |
| | | | | | | |
| Comp. D | 40 | 40 | - | 100 | | phase separation ⁺ |
| 5 | 40 | 20 | 20 | 70 | 1:1 | clear |
| 6 | 40 | 10 | 30 | 40 | 1:3 | clear |
| | | | | | | |
| 7 | 20 | 17.5 | 17.5 | 50 | 1:1 | clear |
| 8 | 25 | 20 | 20 | 60 | 1:1 | clear |

| | | | | | | |
|---|---|---|---|---|---|---|
| + = 20°C storage only | | | | | | |

As can readily be observed, the additive concentrates of the invention, containing both PHGE and PAO, had good storage stability, whilst the comparative examples, containing PHGE alone were insufficiently stable.

### EXAMPLES 9 and 10

A standard VW Polo motor car, equipped with a single carburettor, 4 cylinder, 1.043 litre capacity engine, was used for evaluation of inlet valve cleanliness in a standard road test sequence (Volkswagen Polo Road Test).

Before test inlet parts and combustion chambers were cleaned and new, pre-weighed inlet valves and new spark plugs were fitted to the engine, a new oil filter was fitted and the engine filled with new engine oil. A small wind board was fixed to the roof of the test vehicle to increase wind resistance, and hence engine load. The fuel tank was drained and filled with test gasoline composition prior to operation over a 5000 km test distance. 37 minute test cycles were employed, wherein the vehicle was driven for 30 minutes at 4500 r.p.m. in 4th gear (105 kph) and then allowed to idle for 7 minutes. 12 cycles were covered each day for 8 consecutive days to cover the test distance of 5000 km. At the end of the test, the inlet valves were removed and weighed in order to assess average weight of inlet valve deposits.

Gasoline compositions in accordance with the invention were subject to comparative testing in tests carried out using unleaded gasoline (95 ULG) containing no additives (base gasoline) or containing PMP and either or both of PHGE and PAO. Results are given in Table II following.

**TABLE II**

| Test No. | Concentrations (ppmw) | | | Average inlet valve deposit weight (mg) |
|---|---|---|---|---|
| | PMP | Additive Oil | | |
| | | PHGE | PAO | |
| Comp. E | - | - | - | 387 |
| Example 9 | 250 | 250 | 250 | 31 |
| Comp. F | 250 | 500 | - | 54 |
| Comp. G | 250 | - | 500 | 82 |
| Example 10 | 300 | 200 | 200 | 20 |
| Comp. H | 300 | 300 | - | 44 |

The data in Table II show that in the instances (Examples 9 and 10) where additive oil comprises a combination of PHGE and PAO, weights of deposit on the inlet valves are significantly and surprisingly lower compared with the case where the corresponding amount of additive oil consists solely of one or other PHGE and PAO.

### EXAMPLES 11 to 23

A standard Opel Ascona 1.6 motor car, equipped with a standard 4-cylinder 1.6 litre Type 16SH engine, was used for evaluation of valve sticking by a standard test method.

The test method involved driving the vehicle using a test gasoline composition on normal city roads over a total distance of 130 km over a low-duty cycle (maximum speed 50 kph). The vehicle was then stored overnight at -20°C, and the maximum compression pressure in each cylinder was measured and the average of the four values was calculated. The higher the pressure value, the better the result.

In similar manner to Table II, the compositions of the test gasoline compositions, and the results obtained, are given in Table III following, wherein "additive oil" consisted of PHGE and/or PAO:

**TABLE III**

| Test No. | Concentrations (ppmw) | | Ratio PHGE:PAO (w/w) in Additive Oil | Compression pressure (bar)(x10⁵Pa) |
|---|---|---|---|---|
| | PMP | Additive Oil | | |
| Example 11 | 600 | 1050 | 1:1 | 13.1 |
| | | | | |
| Comp. I | 600 | 1500 | 1:0 | 3:3 |
| Example 12 | 600 | 1500 | 4:1 | 13.3 |
| Example 13 | 600 | 1500 | 1.5:1 | 13.5 |
| Example 14 | 600 | 1500 | 1:1.5 | 12.1 |
| Example 15 | 600 | 1500 | 1:4 | 13.8 |
| Comp. J | 600 | 1500 | 0:1 | 10.3 |
| | | | | |
| Example 16 | 750 | 1200 | 1:1 | 11.1 |
| | | | | |
| Comp. K | 750 | 1500 | 1:0 | 3.8 |
| Example 17 | 750 | 1500 | 4:1 | 7.4 |
| Example 18 | 750 | 1500 | 1.5:1 | 12.9 |
| Example 19 | 750 | 1500 | 1:1.5 | 10.4 |
| Example 20 | 750 | 1500 | 1:4 | 13.3 |
| Comp. L | 750 | 1500 | 0:1 | 13.5 |
| | | | | |
| Comp. M | 900 | 900 | 1:0 | 0.5 |
| Example 21 | 900 | 900 | 1.5:1 | 13.3 |
| Example 22 | 900 | 900 | 1:1 | 13.8 |
| Comp. N | 900 | 900 | 0:1 | 13.4 |
| | | | | |
| Comp. O | 900 | 1200 | 1:0 | 3.5 |
| Example 23 | 900 | 1200 | 1:1 | 13.0 |
| Comp. P | 900 | 1200 | 0:1 | 11.8 |

Those skilled in the art will appreciate that the above concentrations represent three times normal commercial concentrations in order to increase test severity.

The above results show that when the additive oil is a combination of PHGE and PAO, the compression pressure result is very good, always significantly superior to PHGE alone, significantly better than would be predicted for intermediate values between those for PHGE alone and PAO alone, and generally comparable with, and sometimes even superior to those for PAO alone.

### EXAMPLES 24 to 47

The effect of gasoline composition on engine inlet system deposits was assessed by induction system deposit simulator (ISD) testing. In this test method, a gasoline composition was metered to a spray nozzle from which it was expelled in a flat spray pattern onto the surface of an aluminium tube heated to 250°C. The base gasoline used incorporated aged thermally cracked gasoline, in order to encourage formation of deposits. Under the test conditions, such base gasolines alone form a central carbonaceous deposit on the tube surface. Cleanliness-promoting agents prevent deposition in the central area and result in a ring-like deposit on the tube. Residue formation is assessed visually according to the following scale:
0 - clean
1-2 - nearly clean
3-4 - slightly coked
5-6 - medium coked
7-8 - medium to heavily coked
9-10 - heavily coked
over 10 - very heavily coked

In similar manner to Table III, results of the ISD testing are given in Table IV following:

**TABLE IV**

| Test No. | Concentrations (ppmw) | | Ratio PHGE:PAO in Additive Oil | ISD Rating |
|---|---|---|---|---|
| | PMP | Additive Oil | | |
| Example 24 | 100 | 175 | 1:1 | 6 |
| Example 25 | 100 | 200 | 1:1 | 4 |
| | | | | |
| Comp. Q | 100 | 250 | 1:0 | 5 |
| Example 26 | 100 | 250 | 4:1 | 6 |
| Example 27 | 100 | 250 | 1.5:1 | 7 |
| Example 28 | 100 | 250 | 1:1.5 | 6 |
| Example 29 | 100 | 250 | 1:4 | 6 |
| Comp. R | 100 | 250 | 0:1 | 14 |
| | | | | |
| Comp. S | 125 | 250 | 1:0 | 3 |
| Example 30 | 125 | 250 | 4:1 | 3 |
| Example 31 | 125 | 250 | 1.5:1 | 4 |
| Example 32 | 125 | 250 | 1:1.5 | 7 |
| Example 33 | 125 | 250 | 1:4 | 6 |
| Comp. T | 125 | 250 | 0:1 | 14 |
| | | | | |
| Comp. U | 150 | 150 | 1:0 | 2 |
| Example 34 | 150 | 150 | 1:1 | 3 |
| Comp. V | 150 | 150 | 0:1 | 12 |
| | | | | |
| Comp. W | 150 | 200 | 1:0 | 4 |
| Example 35 | 150 | 200 | 1:1 | 3 |
| Comp. X | 150 | 200 | 0:1 | 12 |
| | | | | |
| Example 36 | 200 | 350 | 1:1 | 3 |
| | | | | |
| Comp. Y | 200 | 500 | 1:0 | 2 |
| Example 37 | 200 | 500 | 4:1 | 1 |
| | | | | |
| Example 38 | 200 | 500 | 1.5:1 | 2 |
| Example 39 | 200 | 500 | 1:1.5 | 3 |
| Example 40 | 200 | 500 | 1:4 | 4 |
| Comp. Z | 200 | 500 | 0:1 | 9 |
| | | | | |
| Example 41 | 250 | 400 | 1:1 | 3 |
| | | | | |
| Comp. AA | 250 | 500 | 1:0 | 1 |
| Example 42 | 250 | 500 | 4:1 | 1 |
| Example 43 | 250 | 500 | 1.5:1 | 2 |
| Example 44 | 250 | 500 | 1:1.5 | 3 |
| Example 45 | 250 | 500 | 1:4 | 3 |
| Comp. BB | 250 | 500 | 0:1 | 6 |
| | | | | |
| Comp. CC | 300 | 300 | 1:0 | 1 |
| Example 46 | 300 | 300 | 1:1 | 2 |
| Comp. DD | 300 | 300 | 0:1 | 7 |
| | | | | |
| Comp. EE | 300 | 400 | 1:0 | 1 |
| Example 47 | 300 | 400 | 1:1 | 3 |
| Comp. FF | 300 | 400 | 0:1 | 7 |

The results in Table IV show that when the additive oil is a combination of PHGE and PAO, the ISD rating is generally good, always superior to PAO alone, significantly better than would be predicted for intermediate values between those for PHGE alone and PAO alone, and generally comparable with those for PHGE alone.

In conclusion, it can be noted that additive concentrates containing both PHGE and PAO had good storage stability, by comparision with similar concentrates containing PHGE but not PAO; inlet valve deposits were found to be lower in gasolines containing additive oil in the form of a combination of PHGE and PAO compared with those in which the additive oil was solely PHGE or PAO; avoidance of valve sticking, as evidenced by compression pressure assessment, was significantly superior for combinations of PHGE and PAO than for PHGE alone, and generally comparable to PAO alone; and avoidance of deposit formation, as evidenced by ISD testing, was significantly superior for combinations of PHGE and PAO than for PAO alone, and generally comparable to PHGE alone.

## Claims

1. Gasoline composition comprising a major amount of a gasoline suitable for use in spark-ignition engines, an amount of a polyalphaolefin having a viscosity at 100°C in the range 2 x 10⁻⁶ to 2 x 10⁻⁵ m²/s (2 to 20 centistokes), being a hydrogenated oligomer containing 18 to 80 carbon atoms derived from at least one alphaolefinic monomer containing from 8 to 16 carbon atoms, and an amount of a polyoxyalkylene compound selected from glycols, mono- and diethers thereof, having number average molecular weight (Mₙ) in the range 400 to 3000, the weight ratio polyalphaolefin: polyoxyalkylene compound being in the range 1:10 to 10:1, and the amount of the polyalphaolefin and the polyoxyalkylene compound together being in the range 100 to 1500 ppmw, based on total composition.

2. A composition according to Claim 1 wherein the polyaphaolefin is derived from an alphaolefinic monomer containing from 8 to 12 carbon atoms.

3. A composition according to Claim 1 or 2 wherein the polyalphaolefin has viscosity at 100°C in the range 6 x 10⁻⁶ to 1 x 10⁻⁵m²/s (6 to 10 centistokes).

4. A composition according to any one of Claims 1 to 3 wherein the polyoxyalkylene compound has the formula wherein R¹ and R² independently represent hydrogen atoms or C₁₋₄₀ hydrocarbyl groups, each R independently represents a C₂₋₈ alkylene group and n is such that Mₙ of the polyoxyalkylene compound is in the range 700 to 2000.

5. A composition according to Claim 4 wherein R¹ represents a c₈₋₂₀ alkyl group and R² represents a hydrogen atom.

6. A composition according to Claim 4 or 5 wherein each R independently represents a C₂₋₄ alkylene group.

7. A composition according to any one of Claims 1 to 6 wherein the polyalphaolefin and the polyoxyalkylene compound together are present in an amount in the range 100 to 1200 ppmw, based on total composition.

8. A composition according to any one of Claims 1 to 7 which additionally contains a minor amount of at least one hydrocarbon-soluble ashless dispersant.

9. A composition according to Claim 8 wherein the dispersant comprises a polyolefin-substituted succinimide derivative wherein the polyolefin has Mₙ in the range 800 to 5000.

10. A composition according to Claim 8 or 9 wherein the ashless dispersant is present in an amount in the range 30 to 500 ppmw based on total composition.

11. A composition according to any one of Claims 1 to 10 wherein the weight ratio polyalphaolefin:polyoxyalkylene compound is in the range 1:5 to 5:1.

12. A concentrate suitable for addition to gasoline which comprises a gasoline-compatible diluent, a polyalphaolefin as defined in Claim 1, a polyoxyalkylene compound as defined in Claim 1, the weight ratio polyalphaolefin:polyoxyalkylene compound being in the range 1:10 to 10:1, and optionally also at least one hydrocarbon-soluble ashless dispersant.

13. A concentrate according to Claim 12 wherin the polyalphaolefin and the polyoxyalkylene compound together are present in an amount in the range 20% to 80% w and the ashless dispersant, if present, is present in an amount in the range 5% to 30% w, all percentages being calculated on the diluent.

14. A method of operating a spark-ignition internal combustion engine which comprises introducing into the combustion chambers of said engine a gasoline composition according to any one of Claims 1 to 11.

## Patentansprüche

1. Benzinzusamnensetzung mit einem Gehalt an einer Hauptkomponente aus einem zur Verwendung in fremdgezündeten Motoren geeigneten Benzin, einer Menge eines Polyalphaolefins mit einer Viskosität bei 100°C im Bereich von 2x10⁻⁶ bis 2x10⁻⁵ m²/s (2 bis 20 Centistoke), bei dem es sich um ein hydriertes Oligomer mit 18 bis 80 Kohlenstoffatomen handelt, das von wenigstens einem, 8 bis 16 Kohlenstoffatome enthaltenden alphaolefinischen Monomer abgeleitet ist, und an einer Menge einer unter Glycolen, Mono- und Diethern hievon ausgewählten Polyoxyalkylenverbindung mit einem zahlenmittleren Molekulargewicht (Mₙ) von 400 bis 3.000, wobei das Gewichtsverhältnis Polyalphaolefin; Polyoxylalkylenverbindung im Bereich 1:10 bis 10:1 liegt und die Menge an Polyalphaolefin und Polyoxyalkylenverbindung zusammen im Bereich von 100 bis 1.500 Gewichtsteilen pro Million, bezogen auf die Gesamtzusammensetzung, beträgt.

2. Zusammensetzung nach Anspruch 1, worin das Polyalphaolefin von einem alphaolefinischen Monomer mit 8 bis 12 Kohlenstoffatomen abgeleitet ist.

3. Zusammensetzung nach Anspruch 1 oder 2, worin das Polyalphaolefin eine Viskosität bei 100°C im Bereich von 6x10⁻⁶ bis 1x10⁻⁵ m²/s (6 bis 10 Centistoke) aufweist.

4. Zusammensetzung nach einem der Ansprüche 1 bis 3, worin die Polyoxyalkylenverbindung die Formel aufweist, worin R¹ und R² unabhängig voneinander Wasserßtoffatome oder C₁₋₄₀Hydrocarbylgruppen darstellen, jedes R unabhängig eine C₂-₈A1kylengruppe bedeutet und n eine solche Zahl ist, daß das Mₙ der Polyoxyalkylenverbindung im Bereich von 700 bis 2.000 liegt.

5. Zusammensetzung nach Anspruch 4, worin R¹ eine C₈₋₂₀ Alkylgruppe darstellt und R² für ein Wasserstoffatom steht.

6. Zusammensetzung nach Anspruch 4 oder 5, worin jedes R unabhängig eine C₂₋₄Alkylengruppe bedeutet.

7. Zusammensetzung nach einem der Ansprüche 1 bis 6, worin das Poylalphaolefin und die Polyoxyalkylenverbindung zusammen in einer Menge von 100 bis 1.200 Gewichtsteilen pro Million, bezogen auf die Gesamtzusammensetzung, vorliegen.

8. Zusammensetzung nach einem der Ansprüche 1 bis 7, die zusätzlich eine kleine Menge wenigstens eines kohlenwasserstofflöslichen aschefreien Dispergiermittels enthält.

9. Zusammensetzung nach Anspruch 8, worin das Dispergiermittel ein polyolefinsubstituiertes Succinimidderivat umfaßt, worin das Polyolefin einen Mₙ-Wert im Bereich von 800 bis 5.000 aufweist.

10. Zusammensetzung nach Anspruch 8 oder 9, worin das aschefreie Dispergiermittel in einer Menge im Bereich von 30 bis 500 Gewichtsteilen pro Million, bezogen auf die Gesamtzusasmmensetzung, vorliegt.

11. Zusammensetzung nach einem der Ansprüche 1 bis 10, worin das Gewichtsverhältnis Polyalphaolefin: Polyoxyalkylenverbindung im Bereich 1:5 bis 5:1 liegt.

12. Ein zur Zugabe zu Benzin geeignetes Konzentrat, welches ein benzinverträgliches Verdünnungsmittel, ein Polyalphaolefin, wie in Anspruch 1 definiert, eine Polyoxyalkylenverbindung, wie in Anspruch 1 definiert, wobei das Gewichtsverhältnis Polyalphaolefin: Polyoxyalkylenverbindung im Bereich 1:10 bis 10:1 liegt, und gegebenenfalls auch wenigstens ein kohlenwasserstofflösliches aschefreies Dispergiermittel umfaßt.

13. Konzentrat nach Anspruch 12, worin das Polyalphaolefin und die Polyoxyalkylenverbindung zusammen in einer Menge im Bereich von 20 bis 80 Gew.-% vorliegen und das aschefreie Dispergiermittel, soferne vorhanden, in einer Menge im Bereich von 5 bis 30 Gew.-% vorliegt, wobei alle Prozentsätze auf das verdünnungemittel bezogen sind.

14. Verfahren zum Betreiben einer fremdgezündeten Verbrennungskraftmaschine, welches ein Einführen einer Benzinzusammensetzung nach einem der Ansprüche 1 bis 11 in die Verbrennungsräume dieser Maschine umfaßt.

## Revendications

1. Composition d'essence, qui comprend une quantité majeure d'une essence convenant à l'emploi dans des moteurs à allumage par étincelles, une quantité d'une polyalphaoléfine possédant une viscosité à 100°C qui varie de 2 x 10⁻⁶ à 2 × 10⁻⁵ m²/s (2 à 20 centistokes), étant un oligomère hydrogéné contenant de 18 à 80 atomes de carbone, provenant d'au moins un monomère alphaoléfinique contenant de 2 à 16 atomes de carbone et une quantité d'un composé de polyoxyalkylène choisi parmi les glycols, leurs monoéthers et leurs diéthers, possédant un poids moléculaire moyen en nombre (Mₙ) se situant dans la plage de 400 à 3000, le rapport pondéral polyalphaoléfine:composé de polyoxyalkylène variant dans la plage de 1:10 à 10:1 et la quantité de la polyalphaoléfine et du composé de polyoxyalkylène ensemble fluctuant dans la plage de 100 à 1500 ppm, sur base de la composition totale.

2. Composition suivant la revendication 1, caractérisée en ce que la polyalphaoléfine dérive d'un monomère alphaoléfinique contenant de 8 à 12 atomes de carbone.

3. Composition suivant la revendication 1 ou 2, caractérisée en ce que la polyoléfine possède une viscosité à 100°C qui varie de 6 x 10⁻⁶ à 1 x 10⁻⁵ m²/s (6 à 10 centistokes).

4. Composition suivant l'une quelconque des revendications 1 à 3, caractérisée en ce que le composé de polyoxyalkylène répond à la formule suivante :
R¹-O(̵R-O)̵ₙR² (I)
dans laquelle dans laquelle R¹ et R² représentent chacun indépendamment un atome d'hydrogène ou un radical hydrocarbyle, de préférence, hydrocarbyle en C₁ à C₄₀, chaque symbole R représente indépendamment un radical alkylène en C₂ à C₈ et n est tel que Mₙ du composé de polyoxyalkylène varie dans la plage de 700 à 2000.

5. Composition suivant la revendication 4, caractérisée en ce que R¹ représente un radical alkyle en C₈ à C₂₀ et R² représente un atome d'hydrogène.

6. Composition suivant la revendication 4 ou 5, caractérisée en ce que chaque symbole R représente indépendamment un groupe alkylène en C₂ à C₄.

7. Composition suivant l'une quelconque des revendications 1 à 6, caractérisée en ce que la polyalpholéfine et le composé de polyoxyalkylène ensemble sont présents en une proportion qui varie dans la plage de 100 à 1200 ppmp, sur base de la composition totale.

8. Composition suivant l'une quelconque des revendications 1 à 7, caractérisée en ce qu'elle contient en outre une proportion mineure d'au moins un dispersif sans cendre soluble dans les hydrocarbures.

9. Composition suivant la revendication 8, caractérisée en ce que le dispersif est constitué par un dérivé de succinimide substitué par une polyoléfine, où la polyoléfine possède un Mₙ qui varie de 800 à 5000.

10. Composition suivant la revendication 8 ou 9, caractérisée en ce que le dispersif sans cendre est présent dans la proportion de 30 à 500 ppmp, sur base de la composition totale.

11. Composition suivant l'une quelconque des revendications 1 à 10, caractérisée en ce que le rapport pondéral polyalphaoléfine: composé de polyoxyalkylène varie dans la plage de 1:5 à 5:1.

12. Concentré convenant à l'addition à de l'essence, caractérisé en ce qu'il comprend un diluant compatible avec l'essence, une polyalphaoléfine, telle que définie dans la revendication 1, un composé de polyoxyalkylène, tel que défini dans la revendication 1, le rapport pondéral polyalphaoléfine-composé de polyoxyalkylène variant dans la plage de 1:10 à 10:1 et facultativement aussi, au moins un dispersif sans cendre soluble dans les hydrocarbures.

13. Concentré suivant la revendication 12, caractérisé en ce que la polyalphaoléfine et le composé de polyoxyalkylène ensemble sont présents en une proportion de 20% à 80% p et le dispersif sans cendre, s'il est présent, y est contenu en une proportion de 5% à 30% p, tous les pourcentages étant calculés sur le diluant.

14. Procédé pour faire fonctionner un moteur à combustion inteme à allumage par étincelles, caractérisé en ce que l'on introduit une composition d'essence suivant l'une quelconque des revendications 1 à 11 dans les chambres de combustion dudit moteur.
